

Oct. 16, 1973

TAKESHI MASUYAMA ET AL

3,766,098

VOLTAGE-NONLINEAR RESISTORS

Filed June 22, 1970



TAKESHI MASUYAMA,  
TSUYOSHI NISHI AND  
TOSHIOKI AMEMIYA,  
INVENTORS

BY *Wendoroth, Lund & Ponack*

ATTORNEYS

## 1

3,766,098

### VOLTAGE-NONLINEAR RESISTORS

Takeshi Masuyama and Tsuyoshi Nishi, Osaka, and Toshi-  
oki Amemiya, Tokyo, Japan, assignors to Matsushita  
Electric Industrial Co., Ltd., Kadoma, Osaka, Japan

Filed June 22, 1970, Ser. No. 48,333

Claims priority, application Japan, July 2, 1969,  
44/53,638, 44/53,641; July 4, 1969, 44/54,238,  
44/54,239, 44/54,240; Sept. 1, 1969, 44/70,424,  
44/70,425, 44/70,426, 44/70,427, 44/70,428,  
44/70,429

Int. Cl. H01b 1/06

U.S. CL. 252—519

5 Claims

### ABSTRACT OF THE DISCLOSURE

A voltage nonlinear resistor has a sintered wafer of, as a major part, zinc oxide and, as an additive, iron oxide and one member selected from the group consisting of nickel oxide, titanium oxide, magnesium oxide, manganese oxide, chromium oxide, cobalt oxide, barium oxide, strontium oxide, beryllium oxide, cadmium oxide and lead fluoride. A silver paint electrode is applied to at least one of the opposite surfaces of said sintered wafer.

This invention relates to resistors having a non-linear voltage characteristic, hereinafter called voltage-nonlinear resistors, having non-ohmic resistance, and more particularly relates to varistors comprising zinc oxide with silver electrodes applied thereto.

Various voltage-nonlinear resistors such as silicon carbide varistors, selenium oxide or cuprous oxide rectifiers and germanium or silicon p-n junction diodes, are known. The electrical characteristics of such a voltage-nonlinear resistor are expressed by the relation:

$$I = \left( \frac{V}{C} \right)^n$$

where  $V$  is the voltage across the resistor,  $I$  is the current flowing through the resistor,  $C$  is a constant equivalent to the voltage at a given current and exponent  $n$  is a numerical value greater than 1. The value of  $n$  is calculated by the following equation:

$$n = \frac{\log_{10}(I_2/I_1)}{\log_{10}(V_2/V_1)}$$

where  $V_1$  and  $V_2$  are the voltages at given currents  $I_1$  and  $I_2$ , respectively. Conveniently,  $I_1$  and  $I_2$  are 10 ma. and 100 ma., respectively. The desired value of  $C$  depends upon the kind of application to which the resistor is to be put. It is ordinarily desirable that the value of  $n$  be large as possible since this exponent determines the degree to which the resistors depart from ohmic characteristics.

Silicon carbide varistors are most widely used as voltage-nonlinear resistors and are manufactured by mixing fine particles of silicon carbide with water, ceramic binder and/or conductive material such as graphite or metal powder, pressing the mixture in a mold to the desired shape, and then drying and firing the pressed body in air or a non-oxidizing atmosphere. Silicon carbide varistors with conductive materials are characterized by a low electric resistance, i.e. a low value of  $C$  and a low value of  $n$  whereas silicon carbide varistors without conductive materials have a high electric resistance, i.e. a high value of  $C$  and a high value of  $n$ . It has been difficult to manufacture silicon carbide varistors characterized by a high  $n$  and a low  $C$ . For example, silicon carbide varistors, selenium oxide or cuprous oxide rectifiers exhibit  $n$ -values from 2.5 to 3.3 and  $C$ -values from 6 to 13 at a given current of 100 ma., and silicon carbide varistors without graphite have  $n$ -values from 4 to 7 and  $C$ -values from 30 to 800 at a given current of 1

## 2

ma. with respect to a given size of varistor, e.g. 30 mm. in diameter and 1 mm. in thickness.

Conventional rectifiers comprising selenium oxide or cuprous oxide have an  $n$ -value less than 3 and a  $C$ -value of 5 to 10 at a given current of 100 ma. with respect to a specimen 20 mm. in diameter. In this case, the thickness of sample does not affect the  $C$ -value.

A germanium or silicon p-n junction resistor has an extremely high value of  $n$  but its  $C$ -value is constant, e.g. 10 of the order of 0.7 to 0.3 at a given current of 100 ma. because its diffusion voltage in the V-I characteristic is constant and cannot be changed very greatly. It is necessary for obtaining a desirable  $C$ -value to combine several diodes in series and/or in parallel. Another disadvantage of such diodes is the complicated steps involved in their manufacture, with resultant high cost. As a practical matter, the use of diode resistors is not widespread at the present in view of their high cost even though they may have a high value of  $n$ .

20 An object of this invention is to provide a voltage-nonlinear resistor having a high value of  $n$  and a low value of  $C$ .

A further object of this invention is to provide a voltage-nonlinear resistor capable of being made by a 25 simple manufacturing method which results in a low cost.

A further object of this invention is to provide a voltage-nonlinear resistor characterized by a high stability with respect to temperature, humidity and electric load.

Another object of this invention is to provide a voltage-nonlinear resistor, the  $C$ -value of which can be controlled.

These objects are achieved by providing a voltage-nonlinear resistor which has a sintered wafer of, as a major part, zinc oxide and, as an additive, iron oxide and one member selected from the group consisting of nickel oxide, titanium oxide, magnesium oxide, manganese oxide, chromium oxide, cobalt oxide, barium oxide, beryllium oxide, cadmium oxide and lead fluoride. Electrodes are applied to the opposite surfaces of said sintered wafer, at least one of which electrodes being a silver paint electrode. Leads are then soldered to the electrodes.

These and other objects of the invention will become apparent upon consideration of the following description 45 taken together with the accompanying drawing in which the single figure is a partly cross-sectional view through a voltage-nonlinear resistor in accordance with the invention.

Before proceeding with a detailed description of the 50 voltage-nonlinear resistors contemplated by the invention, their construction will be described with reference to the aforesaid figure of the drawing wherein reference character 10 designates, as a whole, a voltage-nonlinear resistor having, as its active element, a sintered wafer 1 of electrically conductive ceramic material according 55 to the present invention.

Sintered wafer 1 is prepared in a manner hereinafter set forth, and is provided with a pair of electrodes 2 and 3 having specified compositions and applied in a 60 suitable manner hereinafter set forth, on two opposite surfaces of the wafer.

The wafer 1 is a sintered plate having any one of 65 various shapes such as circular, square, rectangular, etc. Wire leads 5 and 6 are attached conductively to the electrodes 2 and 3, respectively, by a connection means 4 (solder or the like).

According to the present invention, sintered wafer 1 consists essentially of, as a major part, zinc oxide and as an additive, iron oxide and one member selected from the group consisting of nickel oxide, titanium oxide, magnesium oxide, manganese oxide, chromium oxide, cobalt oxide, barium oxide, strontium oxide, beryllium oxide,

cadmium oxide and lead fluoride and at least one of electrodes 2 and 3 consists of a silver paint electrode.

Table 1 shows operable and optimal compositions of sintered body 1 for producing a voltage-nonlinear resistor having an *n*-value higher than 7 and a high stability with respect to temperature, humidity and electric load.

Table 2 shows operable and optimal compositions of silver electrodes 2 and 3 after heating for curing in order to produce the novel voltage-nonlinear resistors in accordance with the invention.

Table 3 shows optimal combinations of sintered body 1 and silver electrodes 2 and 3 for producing voltage-nonlinear resistors having a C-value lower than 6 at a given current of 100 ma., an *n*-value higher than 20 and a high stability with respect to temperature, humidity and electric load.

The sintered body 1 can be prepared by a per se well known ceramic technique. The starting materials in having the compositions defined in Table 1 are mixed in a wet mill so as to produce homogeneous mixtures. The mixtures are dried and pressed in a mold into desired shapes at a pressure from 100 kg./cm.<sup>2</sup> to 1000 kg./cm.<sup>2</sup>. The pressed bodies are sintered in air at 1250° C. to 1450° C. for 1 to 3 hours, and then furnace-cooled to room temperature (about 15° to about 30° C.). The pressed bodies are preferably sintered in a non-oxidizing atmosphere such as nitrogen and argon when it is desired to reduce the electrical resistivity. The electrical resistivity also can be reduced by air-quenching from the sintering temperature to room temperature even when the pressed bodies are fired in air.

The iron oxide, nickel oxide, titanium oxide, magnesium oxide, manganese oxide, chromium oxide, cobalt oxide, barium oxide, strontium oxide, beryllium oxide and cadmium oxide which are added to zinc oxide as an additive may be in the form of metal, or carbonate or in any other form which in firing at the temperature employed will be converted to oxide.

The mixtures may be preliminarily calcined at 700 to 1000° C. and pulverized for easy fabrication in the subsequent pressing step. The mixture to be pressed may be admixed with a suitable binder such as water, polyvinyl alcohol, etc.

It is advantageous that the sintered body have the opposite surfaces lapped by abrasive powder such as silicon carbide having a particle size of 300 mesh to 1500 mesh.

The sintered bodies are coated on the opposite surfaces thereof by a silver electrode paint in a per se conventional manner such as by a spray method, screen printing method or brushing method. It is necessary that the silver electrode paint have a solid ingredient composition as defined in Tables 2 and 3 after it is fired at 400° C. to 850° C. in air. Solid ingredients having compositions defined in Table 2 and 3 can be prepared in a per se conventional manner by mixing commercially available powders with organic resin such as epoxy, vinyl and phenol resin in an organic solvent such as butyl acetate, toluene or the like so as to produce silver electrode paints.

The silver powder may be in the form of metallic silver, or in the form of silver carbonate or silver oxide, or in any other form which in firing at the temperatures employed will be converted to metallic silver. Therefore, the term "silver" as used throughout this specification and the claims appended hereto in connection with the silver composition before it is fired, is meant to include silver in any form which in firing will be converted to metallic silver. The viscosity of the resultant silver electrode paints can be controlled by the amounts of resin and solvent. Particle sizes of solid ingredients also are required to be in the range of 0.1 $\mu$  to 5 $\mu$ .

Lead wires can be applied to the silver electrodes in a per se conventional manner by using conventional solder having a low melting point. It is convenient to employ a

conductive adhesive comprising silver powder and resin in an organic solvent for connecting the lead wires to the silver electrodes.

Voltage-nonlinear resistors according to this invention have a high stability with respect to temperature and in a load life test, which is carried out at 70° C. at a rating power for 500 hours. The *n*-value and C-value do not change greatly after heating cycles and the load life test. It is preferable for achieving a high stability to humidity that the resultant voltage-nonlinear resistors be embedded in a humidity proof resin such as epoxy resin and phenol resin in a per se well known manner.

According to the invention, it has been discovered that the method of curing the applied silver electrode paint has a great effect on the *n*-value of the resultant voltage-nonlinear resistor. The *n*-value will not be optimal when the applied silver electrode paint is heated in a non-oxidizing atmosphere such as nitrogen and hydrogen for curing. It is necessary for obtaining a high *n*-value that the applied silver electrode paint be cured by heating in an oxidizing atmosphere such as air and oxygen.

Silver electrodes prepared by any other method than by silver painting result in a poor *n*-value. For example, the sintered body does not become a voltage-nonlinear resistor when it is provided with silver electrodes on the opposite surfaces by electroless plating or electrolytic plating in a conventional manner. Silver electrodes prepared by vacuum evaporation or chemical deposition result in an *n*-value less than 3.

The following examples are given as illustrative of the presently-preferred method of proceeding according to the present invention; however, it is not intended that the scope of said invention be limited to the specific examples.

#### EXAMPLE 1

Respective starting materials according to Table 4 are mixed in a wet mill for 5 hours.

The mixture is dried and pressed in a mold into a disc of 13 mm. diameter and 2.5 mm. thickness at a pressure of 340 kg./cm.<sup>2</sup>.

The pressed body is sintered in air at 1350° C. for 1 hour, and then quenched to room temperature (about 15° to about 30° C.). The sintered disc has the opposite surfaces thereof lapped by silicon carbide with a particle size of 600 mesh. The resulting sintered disc has a size of 10 mm. diameter and 1.5 mm. thickness. The sintered disc is coated on the opposite surfaces thereof with a silver electrode paint by a conventional brushing method. The silver electrode paint employed has a solid ingredient composition according to Table 5 and is prepared by mixing these ingredients with vinyl-resin in amyl acetate. The coated disc is fired at 800° C. for 30 minutes in air.

Lead wires are attached to the silver electrodes by means of silver paint. The electric characteristics of the resultant resistors are shown in Table 4.

#### EXAMPLE 2

Sintered discs having compositions listed in Table 6 are prepared in the same manner as those in Example 1. Each sintered disc has a size of 10 mm. diameter and 1.5 mm. thickness. The sintered disc is coated on one surface thereof with a silver electrode paint having a composition listed in Table 7 in the same manner as that in Example 1 and is then fired at 500° C. in air. Another surface is provided with a spray metallized film of aluminum by a per se well known technique.

Lead wires are attached to the silver electrode and the aluminum electrode by means of conductive silver paint. The electric characteristics of the resultant resistors measured in the easy current flow direction are shown in Table 6.

#### EXAMPLE 3

A sintered disc having a composition of 99.0 mol. percent of zinc oxide, 0.5 mol. percent of iron oxide and 0.5

mol. percent of beryllium oxide is prepared in the same manner as that in Example 1. The sintered disc has a size of 10 mm. diameter and 1.5 mm. thickness. Various silver electrode paints are applied to opposite surfaces of the sintered disc and fired in air at a temperature listed in Table 8. The silver electrode paints have solid ingredient compositions shown in Table 8 and are prepared by mixing 100 weight parts of said solid ingredient compositions with 1 to 20 weight parts of epoxy resin in 20 to 40 weight parts of butyl alcohol. The resultant voltage-nonlinear resistors have desirable C-values and n-values as indicated in Table 8. It will be readily understood that the electrode compositions have a great effect on the electrical characteristics of the resultant voltage-nonlinear resistors.

#### EXAMPLE 4

A sintered disc having a composition of 99.0 mol. percent of zinc oxide, 0.5 mol. percent of iron oxide and 0.5 mol. percent of magnesium oxide is prepared in the same manner as that in Example 1. The sintered disc has a size of 10 mm. diameter and 1.5 mm. thickness. Various silver electrode paints are applied to one surface of the sintered disc and fired in air at a temperature listed in Table 9. The silver electrode paints have solid ingredient compositions shown in Table 9 and are prepared by mixing 100 weight parts of said solid ingredient compositions with 1 to 20 weight parts of epoxy resin in 20 to 40 weight parts of butyl alcohol. Another surface is provided with a nickel electrode by an electroless plating

15

TABLE 1

| Operable composition of sintered body (mol. percent) |                                                                                             |
|------------------------------------------------------|---------------------------------------------------------------------------------------------|
| ZnO                                                  | Additives                                                                                   |
| 99.9 to 80.0                                         | 0.05 to 10.0 Fe <sub>2</sub> O <sub>3</sub> , 0.05 to 10.0 NiO.                             |
| 99.9 to 80.0                                         | 0.05 to 10.0 Fe <sub>2</sub> O <sub>3</sub> , 0.05 to 10.0 TiO <sub>2</sub> .               |
| 99.9 to 80.0                                         | 0.05 to 10.0 Fe <sub>2</sub> O <sub>3</sub> , 0.05 to 10.0 MgO.                             |
| 99.9 to 80.0                                         | 0.05 to 10.0 Fe <sub>2</sub> O <sub>3</sub> , 0.05 to 10.0 MnO.                             |
| 99.9 to 80.0                                         | 0.05 to 10.0 Fe <sub>2</sub> O <sub>3</sub> , 0.05 to 10.0 Cr <sub>2</sub> O <sub>3</sub> . |
| 99.9 to 80.0                                         | 0.05 to 10.0 Fe <sub>2</sub> O <sub>3</sub> , 0.05 to 10.0 CoO.                             |
| 99.9 to 80.0                                         | 0.05 to 10.0 Fe <sub>2</sub> O <sub>3</sub> , 0.05 to 10.0 BaO.                             |
| 99.9 to 80.0                                         | 0.05 to 10.0 Fe <sub>2</sub> O <sub>3</sub> , 0.05 to 10.0 SrO.                             |
| 99.9 to 80.0                                         | 0.05 to 10.0 Fe <sub>2</sub> O <sub>3</sub> , 0.05 to 10.0 BeO.                             |
| 99.0 to 80.0                                         | 0.05 to 10.0 Fe <sub>2</sub> O <sub>3</sub> , 0.05 to 10.0 CdO.                             |
| 99.9 to 80.0                                         | 0.05 to 10.0 Fe <sub>2</sub> O <sub>3</sub> , 0.05 to 10.0 PbF <sub>2</sub> .               |

| Optimal composition of sintered body (mol. percent) |                                                                                         |
|-----------------------------------------------------|-----------------------------------------------------------------------------------------|
| 99.8 to 94.0                                        | 0.1 to 3.0 Fe <sub>2</sub> O <sub>3</sub> , 0.1 to 3.0 NiO.                             |
| 99.9 to 94.0                                        | 0.1 to 3.0 Fe <sub>2</sub> O <sub>3</sub> , 0.1 to 3.0 TiO <sub>2</sub> .               |
| 99.8 to 94.0                                        | 0.1 to 3.0 Fe <sub>2</sub> O <sub>3</sub> , 0.1 to 3.0 MgO.                             |
| 99.8 to 94.0                                        | 0.1 to 3.0 Fe <sub>2</sub> O <sub>3</sub> , 0.1 to 3.0 MnO.                             |
| 99.8 to 94.0                                        | 0.1 to 3.0 Fe <sub>2</sub> O <sub>3</sub> , 0.1 to 3.0 Cr <sub>2</sub> O <sub>3</sub> . |
| 99.8 to 94.0                                        | 0.1 to 3.0 Fe <sub>2</sub> O <sub>3</sub> , 0.1 to 3.0 CoO.                             |
| 99.8 to 94.0                                        | 0.1 to 3.0 Fe <sub>2</sub> O <sub>3</sub> , 0.1 to 3.0 BaO.                             |
| 99.8 to 94.0                                        | 0.1 to 3.0 Fe <sub>2</sub> O <sub>3</sub> , 0.1 to 3.0 SrO.                             |
| 99.8 to 94.0                                        | 0.1 to 3.0 Fe <sub>2</sub> O <sub>3</sub> , 0.1 to 3.0 BeO.                             |
| 99.8 to 94.0                                        | 0.1 to 3.0 Fe <sub>2</sub> O <sub>3</sub> , 0.1 to 3.0 CdO.                             |
| 99.8 to 94.0                                        | 0.1 to 3.0 Fe <sub>2</sub> O <sub>3</sub> , 0.1 to 3.0 PbF <sub>2</sub> .               |

TABLE 2

| Operable composition of electrode (wt. percent) |             |                                |                  |                               |          |          |
|-------------------------------------------------|-------------|--------------------------------|------------------|-------------------------------|----------|----------|
| Ag                                              | PbO         | Bi <sub>2</sub> O <sub>3</sub> | SiO <sub>2</sub> | B <sub>2</sub> O <sub>3</sub> | CoO      | MnO      |
| 70.0 to 99.0                                    | 1.0 to 20.0 | 0 to 10                        | 0 to 10          | 0 to 10                       | 0 to 6.0 |          |
| 70.0 to 99.0                                    |             | 1.0 to 20.0                    | 0 to 10          | 0 to 10                       | 0 to 6.0 |          |
| 70.0 to 99.0                                    | 1 to 20.0   | 0 to 10                        | 0 to 10          | 0 to 10                       |          | 0 to 6.0 |
| 70.0 to 99.0                                    |             | 1.0 to 30.0                    | 0 to 10          | 0 to 10                       |          | 0 to 6.0 |

  

| Optimal composition of electrode (wt. percent) |              |            |            |             |  |  |
|------------------------------------------------|--------------|------------|------------|-------------|--|--|
| 75.0 to 95.0                                   | 2.95 to 15.0 | 1.0 to 5.0 | 1.0 to 5.0 | 0.05 to 3.0 |  |  |
| 75.0 to 95.0                                   | 2.95 to 15.0 | 1.0 to 5.0 | 1.0 to 5.0 | 0.05 to 3.0 |  |  |
| 76.0 to 95.0                                   | 2.95 to 15.0 | 1.0 to 5.0 | 1.0 to 5.0 | 0.05 to 3.0 |  |  |
| 75.0 to 95.0                                   | 2.95 to 15.0 | 1.0 to 5.0 | 1.0 to 5.0 | 0.05 to 3.0 |  |  |

TABLE 3  
[Optimal combinations of sintered body and electrode]

| Composition of Sintered Body<br>(mol. percent) |                                                               | Composition of Electrode (wt. percent) |                                |                  |                               |            |
|------------------------------------------------|---------------------------------------------------------------|----------------------------------------|--------------------------------|------------------|-------------------------------|------------|
| ZnO                                            | Additive                                                      | Ag                                     | Bi <sub>2</sub> O <sub>3</sub> | SiO <sub>2</sub> | B <sub>2</sub> O <sub>3</sub> | CoO        |
| 98.0 to 94.0                                   | {0.1 to 3.0 Fe <sub>2</sub> O <sub>3</sub> } {0.1 to 3.0 NiO} | 80.0 to 90.0                           | 7.0 to 14.0                    | 1.0 to 4.0       | 1.0 to 4.0                    | 1.0 to 4.0 |

method. The resultant voltage-nonlinear resistors have desirable C-values and n-values as indicated in Table 9.

#### EXAMPLE 5

The resistors of Example 1 and Example 2 are tested according to the methods used in testing electronic component parts. The load life test is carried out at 70° C. ambient temperature at 1 and 2 watts rating power for 500 hours. The heating cycle test is carried out by repeating 5 times a cycle in which said resistors are kept at 85° C. ambient temperature for 30 minutes, cooled rapidly to -20° C. and then kept at such temperature for 30 minutes. After heating cycle and load life tests, the change rates in the C-value and n-value are as shown in Table 10.

#### EXAMPLE 6

Zinc oxide sintered discs having additives in the amounts listed in Table 11 are prepared in the same manner as that in Example 1. Silver electrode paints having a solid ingredient compositions listed in Table 11 are coated on opposite surfaces of the respective sintered discs in the same manner as that in Example 1 and are fired at 800° C. in air. The electrical characteristics of the resultant voltage-nonlinear resistors are shown in Table 11.

55

TABLE 4

| Starting materials (mol. percent) |                                                                          | Electric characteristics of resultant resistors |      |
|-----------------------------------|--------------------------------------------------------------------------|-------------------------------------------------|------|
| ZnO                               | Additives                                                                | C (at a given current of 100 ma.)               | n    |
| 99.9                              | Fe <sub>2</sub> O <sub>3</sub> 0.05, NiO 0.05                            | 2.6                                             | 7.2  |
| 99.8                              | Fe <sub>2</sub> O <sub>3</sub> 0.1, NiO 0.1                              | 4.2                                             | 10.4 |
| 96.9                              | Fe <sub>2</sub> O <sub>3</sub> 0.1, NiO 3.0                              | 4.7                                             | 13.2 |
| 94.0                              | Fe <sub>2</sub> O <sub>3</sub> 3.0, NiO 3.0                              | 5.3                                             | 11.8 |
| 80.0                              | Fe <sub>2</sub> O <sub>3</sub> 10.0, NiO 10.0                            | 6.4                                             | 7.5  |
| 99.9                              | Fe <sub>2</sub> O <sub>3</sub> 0.05, TiO <sub>2</sub> 0.05               | 2.5                                             | 7.0  |
| 99.8                              | Fe <sub>2</sub> O <sub>3</sub> 0.1, TiO <sub>2</sub> 0.1                 | 3.8                                             | 10.0 |
| 96.9                              | Fe <sub>2</sub> O <sub>3</sub> 0.1, TiO <sub>2</sub> 3.0                 | 4.2                                             | 11.4 |
| 94.0                              | Fe <sub>2</sub> O <sub>3</sub> 3.0, TiO <sub>2</sub> 3.0                 | 4.7                                             | 10.8 |
| 80.0                              | Fe <sub>2</sub> O <sub>3</sub> 10.0, TiO <sub>2</sub> 10.0               | 6.4                                             | 7.2  |
| 99.9                              | Fe <sub>2</sub> O <sub>3</sub> 0.05, MgO 0.05                            | 2.8                                             | 7.8  |
| 99.8                              | Fe <sub>2</sub> O <sub>3</sub> 0.1, MgO 0.1                              | 3.9                                             | 12.6 |
| 96.9                              | Fe <sub>2</sub> O <sub>3</sub> 0.1, MgO 3.0                              | 4.5                                             | 15.4 |
| 94.0                              | Fe <sub>2</sub> O <sub>3</sub> 3.0, MgO 3.0                              | 5.7                                             | 11.8 |
| 80.0                              | Fe <sub>2</sub> O <sub>3</sub> 10.0, MgO 10.0                            | 7.2                                             | 8.5  |
| 99.9                              | Fe <sub>2</sub> O <sub>3</sub> 0.05, MnO 0.05                            | 3.4                                             | 7.1  |
| 99.8                              | Fe <sub>2</sub> O <sub>3</sub> 0.1, MnO 0.1                              | 4.5                                             | 10.4 |
| 96.9                              | Fe <sub>2</sub> O <sub>3</sub> 0.1, MnO 3.0                              | 5.2                                             | 11.6 |
| 94.0                              | Fe <sub>2</sub> O <sub>3</sub> 3.0, MnO 3.0                              | 5.3                                             | 11.5 |
| 80.0                              | Fe <sub>2</sub> O <sub>3</sub> 10.0, MnO 10.0                            | 7.5                                             | 7.0  |
| 99.9                              | Fe <sub>2</sub> O <sub>3</sub> 0.05, Cr <sub>2</sub> O <sub>3</sub> 0.05 | 2.8                                             | 7.4  |
| 99.8                              | Fe <sub>2</sub> O <sub>3</sub> 0.1, Cr <sub>2</sub> O <sub>3</sub> 0.1   | 4.5                                             | 10.3 |
| 96.9                              | Fe <sub>2</sub> O <sub>3</sub> 0.1, Cr <sub>2</sub> O <sub>3</sub> 3.0   | 5.1                                             | 11.4 |
| 94.0                              | Fe <sub>2</sub> O <sub>3</sub> 3.0, Cr <sub>2</sub> O <sub>3</sub> 3.0   | 5.8                                             | 11.2 |
| 80.0                              | Fe <sub>2</sub> O <sub>3</sub> 10.0, Cr <sub>2</sub> O <sub>3</sub> 10.0 | 6.4                                             | 7.9  |
| 99.9                              | Fe <sub>2</sub> O <sub>3</sub> 0.05, CoO 0.05                            | 3.8                                             | 8.5  |
| 99.8                              | Fe <sub>2</sub> O <sub>3</sub> 0.1, CoO 0.1                              | 4.5                                             | 14.3 |

75

7 TABLE 4—Continued

| Starting materials (mol. percent) |                                                            | Electric characteristics of resultant resistors |      |    |
|-----------------------------------|------------------------------------------------------------|-------------------------------------------------|------|----|
| ZnO                               | Additives                                                  | C (at a given current of 100 ma.)               | n    | 5  |
| 96.9                              | Fe <sub>2</sub> O <sub>3</sub> 0.1, CoO 3.0                | 4.9                                             | 15.2 |    |
| 94.0                              | Fe <sub>2</sub> O <sub>3</sub> 3.0, CoO 3.0                | 4.7                                             | 11.4 |    |
| 80.0                              | Fe <sub>2</sub> O <sub>3</sub> 10.0, CoO 10.0              | 6.4                                             | 8.8  |    |
| 99.9                              | Fe <sub>2</sub> O <sub>3</sub> 0.05, BaO 0.05              | 3.2                                             | 7.3  |    |
| 99.8                              | Fe <sub>2</sub> O <sub>3</sub> 0.1, BaO 0.1                | 3.9                                             | 10.0 |    |
| 96.9                              | Fe <sub>2</sub> O <sub>3</sub> 0.1, BaO 3.0                | 4.6                                             | 11.5 | 10 |
| 94.0                              | Fe <sub>2</sub> O <sub>3</sub> 3.0, BaO 3.0                | 5.2                                             | 12.3 |    |
| 80.0                              | Fe <sub>2</sub> O <sub>3</sub> 10.0, BaO 10.0              | 8.4                                             | 8.2  |    |
| 99.9                              | Fe <sub>2</sub> O <sub>3</sub> 0.05, SrO 0.05              | 2.8                                             | 7.4  |    |
| 99.8                              | Fe <sub>2</sub> O <sub>3</sub> 0.1, SrO 0.1                | 3.5                                             | 10.3 |    |
| 96.9                              | Fe <sub>2</sub> O <sub>3</sub> 0.1, SrO 3.0                | 4.2                                             | 11.3 |    |
| 94.0                              | Fe <sub>2</sub> O <sub>3</sub> 3.0, SrO 3.0                | 4.6                                             | 12.7 |    |
| 96.9                              | Fe <sub>2</sub> O <sub>3</sub> 3.0, SrO 0.1                | 5.4                                             | 12.4 | 15 |
| 80.0                              | Fe <sub>2</sub> O <sub>3</sub> 10.0, SrO 10.0              | 6.3                                             | 8.1  |    |
| 99.9                              | Fe <sub>2</sub> O <sub>3</sub> 0.05, BeO 0.05              | 2.4                                             | 7.1  |    |
| 99.8                              | Fe <sub>2</sub> O <sub>3</sub> 0.1, BeO 0.1                | 3.2                                             | 10.0 |    |
| 96.9                              | Fe <sub>2</sub> O <sub>3</sub> 0.1, BeO 3.0                | 4.4                                             | 10.4 |    |
| 94.0                              | Fe <sub>2</sub> O <sub>3</sub> 3.0, BeO 3.0                | 5.3                                             | 10.8 |    |
| 96.9                              | Fe <sub>2</sub> O <sub>3</sub> 3.0, BeO 0.1                | 5.6                                             | 10.5 |    |
| 80.0                              | Fe <sub>2</sub> O <sub>3</sub> 10.0, BeO 10.0              | 6.2                                             | 8.0  |    |
| 99.9                              | Fe <sub>2</sub> O <sub>3</sub> 0.05, CdO 0.05              | 3.5                                             | 7.8  | 20 |
| 99.8                              | Fe <sub>2</sub> O <sub>3</sub> 0.1, CdO 0.1                | 3.9                                             | 10.3 |    |
| 96.9                              | Fe <sub>2</sub> O <sub>3</sub> 0.1, CdO 3.0                | 4.2                                             | 11.6 |    |
| 94.0                              | Fe <sub>2</sub> O <sub>3</sub> 3.0, CdO 3.0                | 5.3                                             | 11.2 |    |
| 96.9                              | Fe <sub>2</sub> O <sub>3</sub> 3.0, CdO 0.1                | 4.8                                             | 10.5 |    |
| 80.0                              | Fe <sub>2</sub> O <sub>3</sub> 10.0, CdO 10.0              | 3.4                                             | 7.1  |    |
| 99.9                              | Fe <sub>2</sub> O <sub>3</sub> 0.05, PbF <sub>2</sub> 0.05 | 3.7                                             | 7.5  |    |
| 99.8                              | Fe <sub>2</sub> O <sub>3</sub> 0.1, PbF <sub>2</sub> 0.1   | 4.5                                             | 11.6 | 25 |
| 96.9                              | Fe <sub>2</sub> O <sub>3</sub> 0.1, PbF <sub>2</sub> 3.0   | 4.7                                             | 13.4 |    |
| 94.0                              | Fe <sub>2</sub> O <sub>3</sub> 3.0, PbF <sub>2</sub> 3.0   | 5.2                                             | 14.5 |    |
| 96.9                              | Fe <sub>2</sub> O <sub>3</sub> 3.0, PbF <sub>2</sub> 0.1   | 6.3                                             | 11.3 |    |
| 80.0                              | Fe <sub>2</sub> O <sub>3</sub> 10.0, PbF <sub>2</sub> 10.0 | 7.4                                             | 8.2  |    |

TABLE 5  
Composition of silver electrode (wt. percent)

| Ag | Bi <sub>2</sub> O <sub>3</sub> | SiO <sub>2</sub> | B <sub>2</sub> O <sub>3</sub> |
|----|--------------------------------|------------------|-------------------------------|
| 80 | 14                             | 4                | 2                             |

TABLE 6

| Starting materials (mol. percent) |                                                            | Electric characteristics of resultant resistors |      |    |
|-----------------------------------|------------------------------------------------------------|-------------------------------------------------|------|----|
| ZnO                               | Additives                                                  | C (at a given current of 100 ma.)               | n    | 40 |
| 99.9                              | Fe <sub>2</sub> O <sub>3</sub> 0.05, NiO 0.05              | 0.6                                             | 15.3 |    |
| 99.8                              | Fe <sub>2</sub> O <sub>3</sub> 0.1, NiO 0.1                | 0.6                                             | 17.8 |    |
| 96.9                              | Fe <sub>2</sub> O <sub>3</sub> 0.1, NiO 3.0                | 0.7                                             | 18.6 |    |
| 94.0                              | Fe <sub>2</sub> O <sub>3</sub> 3.0, NiO 3.0                | 0.7                                             | 18.4 |    |
| 80.0                              | Fe <sub>2</sub> O <sub>3</sub> 10.0, NiO 10.0              | 0.8                                             | 15.7 |    |
| 99.9                              | Fe <sub>2</sub> O <sub>3</sub> 0.05, TiO <sub>2</sub> 0.05 | 0.6                                             | 15.5 |    |
| 99.8                              | Fe <sub>2</sub> O <sub>3</sub> 0.1, TiO <sub>2</sub> 0.1   | 0.6                                             | 17.6 | 45 |
| 96.9                              | Fe <sub>2</sub> O <sub>3</sub> 0.1, TiO <sub>2</sub> 3.0   | 0.7                                             | 18.2 |    |
| 94.0                              | Fe <sub>2</sub> O <sub>3</sub> 3.0, TiO <sub>2</sub> 3.0   | 0.8                                             | 18.3 |    |

TABLE 6—Continued

| Starting materials (mol. percent) |                                                                          | Electric characteristics of resultant resistors |      |   |
|-----------------------------------|--------------------------------------------------------------------------|-------------------------------------------------|------|---|
| ZnO                               | Additives                                                                | C (at a given current of 100 ma.)               | n    | 5 |
| 80.0                              | Fe <sub>2</sub> O <sub>3</sub> 10.0, TiO <sub>2</sub> 10.0               | 0.8                                             | 15.3 |   |
| 99.9                              | Fe <sub>2</sub> O <sub>3</sub> 0.05, MgO 0.05                            | 0.6                                             | 16.4 |   |
| 99.8                              | Fe <sub>2</sub> O <sub>3</sub> 0.1, MgO 0.1                              | 0.7                                             | 17.6 |   |
| 96.9                              | Fe <sub>2</sub> O <sub>3</sub> 0.1, MgO 3.0                              | 0.8                                             | 18.8 |   |
| 94.0                              | Fe <sub>2</sub> O <sub>3</sub> 3.0, MgO 3.0                              | 0.8                                             | 18.2 |   |
| 80.0                              | Fe <sub>2</sub> O <sub>3</sub> 10.0, MgO 10.0                            | 0.8                                             | 15.2 |   |
| 99.9                              | Fe <sub>2</sub> O <sub>3</sub> 0.05, MnO 0.05                            | 0.6                                             | 16.4 |   |
| 99.8                              | Fe <sub>2</sub> O <sub>3</sub> 0.1, MnO 0.1                              | 0.8                                             | 18.6 |   |
| 96.9                              | Fe <sub>2</sub> O <sub>3</sub> 0.1, MnO 3.0                              | 0.8                                             | 18.4 |   |
| 94.0                              | Fe <sub>2</sub> O <sub>3</sub> 3.0, MnO 3.0                              | 0.8                                             | 18.8 |   |
| 80.0                              | Fe <sub>2</sub> O <sub>3</sub> 10.0, MnO 10.0                            | 0.8                                             | 15.7 |   |
| 99.9                              | Fe <sub>2</sub> O <sub>3</sub> 0.05, Cr <sub>2</sub> O <sub>3</sub> 0.05 | 0.6                                             | 16.2 |   |
| 99.8                              | Fe <sub>2</sub> O <sub>3</sub> 0.1, Cr <sub>2</sub> O <sub>3</sub> 0.1   | 0.7                                             | 17.8 |   |
| 96.9                              | Fe <sub>2</sub> O <sub>3</sub> 0.1, Cr <sub>2</sub> O <sub>3</sub> 3.0   | 0.8                                             | 18.5 |   |
| 94.0                              | Fe <sub>2</sub> O <sub>3</sub> 3.0, Cr <sub>2</sub> O <sub>3</sub> 3.0   | 0.7                                             | 18.7 |   |
| 80.0                              | Fe <sub>2</sub> O <sub>3</sub> 10.0, Cr <sub>2</sub> O <sub>3</sub> 10.0 | 0.8                                             | 16.4 |   |
| 99.9                              | Fe <sub>2</sub> O <sub>3</sub> 0.05, CoO 0.05                            | 0.6                                             | 15.5 |   |
| 99.8                              | Fe <sub>2</sub> O <sub>3</sub> 0.1, CoO 0.1                              | 0.7                                             | 17.5 |   |
| 96.9                              | Fe <sub>2</sub> O <sub>3</sub> 0.1, CoO 3.0                              | 0.8                                             | 17.9 |   |
| 94.0                              | Fe <sub>2</sub> O <sub>3</sub> 3.0, CoO 3.0                              | 0.7                                             | 17.2 |   |
| 80.0                              | Fe <sub>2</sub> O <sub>3</sub> 10.0, CoO 10.0                            | 0.6                                             | 16.3 |   |
| 99.9                              | Fe <sub>2</sub> O <sub>3</sub> 0.05, BaO 0.05                            | 0.6                                             | 15.3 |   |
| 99.8                              | Fe <sub>2</sub> O <sub>3</sub> 0.1, SrO 0.05                             | 0.7                                             | 15.2 |   |
| 96.9                              | Fe <sub>2</sub> O <sub>3</sub> 0.1, SrO 0.1                              | 0.7                                             | 17.7 |   |
| 94.0                              | Fe <sub>2</sub> O <sub>3</sub> 3.0, SrO 3.0                              | 0.8                                             | 17.7 |   |
| 80.0                              | Fe <sub>2</sub> O <sub>3</sub> 10.0, SrO 10.0                            | 0.6                                             | 15.5 |   |
| 99.9                              | Fe <sub>2</sub> O <sub>3</sub> 0.05, BeO 0.05                            | 0.6                                             | 16.7 |   |
| 99.8                              | Fe <sub>2</sub> O <sub>3</sub> 0.1, BeO 0.1                              | 0.8                                             | 18.3 |   |
| 96.9                              | Fe <sub>2</sub> O <sub>3</sub> 0.1, BeO 3.0                              | 0.8                                             | 18.9 |   |
| 94.0                              | Fe <sub>2</sub> O <sub>3</sub> 3.0, BeO 3.0                              | 0.8                                             | 18.2 |   |
| 96.9                              | Fe <sub>2</sub> O <sub>3</sub> 0.1, BeO 0.1                              | 0.8                                             | 18.3 |   |
| 94.0                              | Fe <sub>2</sub> O <sub>3</sub> 10.0, BeO 10.0                            | 0.7                                             | 16.1 |   |
| 99.9                              | Fe <sub>2</sub> O <sub>3</sub> 0.05, CdO 0.05                            | 0.6                                             | 15.4 |   |
| 99.8                              | Fe <sub>2</sub> O <sub>3</sub> 0.1, CdO 0.1                              | 0.7                                             | 17.7 |   |
| 96.9                              | Fe <sub>2</sub> O <sub>3</sub> 0.1, CdO 3.0                              | 0.8                                             | 18.4 |   |
| 94.0                              | Fe <sub>2</sub> O <sub>3</sub> 3.0, CdO 3.0                              | 0.8                                             | 18.6 |   |
| 96.9                              | Fe <sub>2</sub> O <sub>3</sub> 0.1, CdO 0.1                              | 0.8                                             | 18.9 |   |
| 94.0                              | Fe <sub>2</sub> O <sub>3</sub> 10.0, CdO 10.0                            | 0.6                                             | 15.6 |   |
| 99.9                              | Fe <sub>2</sub> O <sub>3</sub> 0.05, PbF <sub>2</sub> 0.05               | 0.6                                             | 15.7 |   |
| 99.8                              | Fe <sub>2</sub> O <sub>3</sub> 0.1, PbF <sub>2</sub> 0.1                 | 0.7                                             | 18.2 |   |
| 96.9                              | Fe <sub>2</sub> O <sub>3</sub> 0.1, PbF <sub>2</sub> 3.0                 | 0.8                                             | 18.9 |   |
| 94.0                              | Fe <sub>2</sub> O <sub>3</sub> 3.0, PbF <sub>2</sub> 3.0                 | 0.8                                             | 18.8 |   |
| 96.9                              | Fe <sub>2</sub> O <sub>3</sub> 3.0, PbF <sub>2</sub> 0.1                 | 0.8                                             | 18.9 |   |
| 80.0                              | Fe <sub>2</sub> O <sub>3</sub> 10.0, PbF <sub>2</sub> 10.0               | 0.8                                             | 15.8 |   |

TABLE 7

| Composition of silver electrode (wt. percent) |     |                  |                               |
|-----------------------------------------------|-----|------------------|-------------------------------|
| Ag                                            | PbO | SiO <sub>2</sub> | B <sub>2</sub> O <sub>3</sub> |
| 80                                            | 14  | 4                | 2                             |

| The characteristics of the resultant resistors |      |                                |                  |                               |     |     |
|------------------------------------------------|------|--------------------------------|------------------|-------------------------------|-----|-----|
| Ag                                             | PbO  | Bi <sub>2</sub> O <sub>3</sub> | SiO <sub>2</sub> | B <sub>2</sub> O <sub>3</sub> | CoO | MnO |
| 70                                             | 20   | 10                             | 0                | 0                             | 600 | 5.2 |
| 70                                             | 20   | 0                              | 10               | 5                             | 600 | 4.8 |
| 70                                             | 20   | 5                              | 5                | 6                             | 600 | 5.3 |
| 70                                             | 20   | 4                              | 6                | 6                             | 600 | 5.6 |
| 70                                             | 20   | 4                              | 6                | 6                             | 600 | 5.5 |
| 70                                             | 20   | 4                              | 6                | 6                             | 600 | 6.2 |
| 70                                             | 20   | 4                              | 6                | 6                             | 600 | 6.4 |
| 75                                             | 15   | 5                              | 2                | 3                             | 600 | 4.8 |
| 75                                             | 15   | 2                              | 5                | 3                             | 600 | 5.2 |
| 75                                             | 15   | 5                              | 2                | 3                             | 600 | 6.3 |
| 75                                             | 15   | 2                              | 5                | 3                             | 600 | 6.4 |
| 95                                             | 2.95 | 1.0                            | 1.0              | 0.05                          | 600 | 4.5 |
| 95                                             | 2.95 | 1.0                            | 1.0              | 0.05                          | 600 | 5.2 |
| 99                                             | 1.0  | 0                              | 0                | 0                             | 600 | 3.8 |
| 70                                             | 20   | 10                             | 0                | 0                             | 800 | 4.3 |
| 70                                             | 20   | 0                              | 10               | 5                             | 800 | 4.6 |
| 70                                             | 20   | 5                              | 5                | 6                             | 800 | 5.2 |
| 70                                             | 20   | 4                              | 6                | 6                             | 800 | 4.6 |
| 70                                             | 20   | 4                              | 6                | 6                             | 800 | 4.8 |
| 70                                             | 20   | 4                              | 6                | 6                             | 800 | 5.4 |
| 70                                             | 20   | 4                              | 6                | 6                             | 800 | 5.8 |
| 75                                             | 15   | 5                              | 2                | 3                             | 800 | 5.2 |
| 75                                             | 15   | 2                              | 5                | 3                             | 800 | 4.6 |
| 75                                             | 15   | 5                              | 2                | 3                             | 800 | 4.7 |
| 75                                             | 15   | 2                              | 5                | 3                             | 800 | 6.0 |
| 95                                             | 2.95 | 1.0                            | 1.0              | 0.05                          | 800 | 5.2 |
| 95                                             | 2.95 | 1.0                            | 1.0              | 0.05                          | 800 | 4.4 |
| 99                                             | 1.0  | 0                              | 0                | 0                             | 800 | 4.0 |
| 80                                             | 10   | 5                              | 5                | 5                             | 400 | 3.2 |
| 80                                             | 10   | 5                              | 5                | 5                             | 550 | 3.6 |
| 80                                             | 10   | 5                              | 5                | 5                             | 650 | 4.2 |
| 80                                             | 10   | 5                              | 5                | 5                             | 750 | 4.8 |
| 80                                             | 10   | 5                              | 5                | 5                             | 850 | 5.6 |

TABLE 9

| Composition of electrode (wt. percent) |      |                                |                  |                               |      |      | The characteristics of the resultant resistors |                                   |      |
|----------------------------------------|------|--------------------------------|------------------|-------------------------------|------|------|------------------------------------------------|-----------------------------------|------|
| Ag                                     | PbO  | Bi <sub>2</sub> O <sub>3</sub> | SiO <sub>2</sub> | B <sub>2</sub> O <sub>3</sub> | CoO  | MnO  | Firing temperature of electrode (°C.)          | C (at a given current of 100 mA.) | n    |
| 70                                     | 20   |                                | 10               | 0                             |      |      | 500                                            | 0.8                               | 18.2 |
| 70                                     | 20   |                                | 0                | 10                            |      |      | 500                                            | 0.8                               | 18.4 |
| 70                                     | 20   |                                | 5                | 5                             |      |      | 500                                            | 0.7                               | 18.8 |
| 70                                     | 20   |                                |                  | 4                             | 6    |      | 500                                            | 0.8                               | 18.8 |
| 70                                     | 20   |                                |                  |                               | 6    |      | 500                                            | 0.8                               | 18.7 |
| 70                                     | 20   |                                | 4                | 4                             |      | 6    | 500                                            | 0.7                               | 18.9 |
| 70                                     | 20   |                                |                  |                               |      | 6    | 500                                            | 0.8                               | 18.5 |
| 75                                     | 15   |                                | 5                | 2                             | 3    |      | 500                                            | 0.8                               | 21.4 |
| 75                                     | 15   |                                | 2                | 5                             | 3    |      | 500                                            | 0.8                               | 22.1 |
| 75                                     | 15   |                                | 2                | 5                             |      | 3    | 500                                            | 0.8                               | 23.3 |
| 75                                     | 15   |                                |                  | 5                             |      | 3    | 600                                            | 0.8                               | 22.2 |
| 95                                     | 2.95 |                                | 1.0              | 1.0                           | 0.05 |      | 500                                            | 0.7                               | 21.5 |
| 95                                     | 2.95 |                                | 1.0              | 1.0                           |      | 0.05 | 500                                            | 0.7                               | 21.0 |
| 99                                     | 1.0  |                                |                  |                               |      |      | 500                                            | 0.7                               | 17.4 |
| 70                                     |      | 20                             | 10               | 0                             |      |      | 600                                            | 0.8                               | 17.4 |
| 70                                     |      | 20                             | 0                | 10                            |      |      | 600                                            | 0.7                               | 17.2 |
| 70                                     |      | 20                             | 5                | 5                             |      |      | 600                                            | 0.7                               | 16.8 |
| 70                                     |      | 20                             |                  | 4                             |      |      | 600                                            | 0.8                               | 17.4 |
| 70                                     |      | 20                             | 4                |                               | 6    |      | 600                                            | 0.8                               | 18.2 |
| 70                                     |      | 20                             |                  | 4                             | 6    |      | 600                                            | 0.8                               | 17.3 |
| 70                                     |      | 20                             | 4                |                               |      | 6    | 600                                            | 0.8                               | 17.5 |
| 75                                     |      | 15                             | 5                | 2                             | 3    | 6    | 600                                            | 0.8                               | 20.3 |
| 75                                     |      | 15                             | 2                | 5                             | 3    |      | 600                                            | 0.8                               | 21.2 |
| 75                                     |      | 15                             | 5                | 2                             |      | 3    | 600                                            | 0.8                               | 20.4 |
| 75                                     |      | 15                             | 2                | 5                             |      | 3    | 600                                            | 0.8                               | 20.6 |
| 95                                     | 2.95 |                                | 1.0              | 1.0                           | 0.05 |      | 600                                            | 0.8                               | 20.0 |
| 95                                     | 2.95 |                                | 1.0              | 1.0                           |      | 0.05 | 600                                            | 0.7                               | 21.3 |
| 99                                     | 1.0  |                                |                  |                               |      |      | 600                                            | 0.7                               | 21.4 |
| 80                                     | 10   |                                | 5                | 5                             |      |      | 400                                            | 0.6                               | 18.4 |
| 80                                     | 10   |                                |                  | 5                             |      |      | 550                                            | 0.7                               | 18.2 |
| 80                                     | 10   |                                | 5                | 5                             |      |      | 650                                            | 0.8                               | 17.3 |
| 80                                     | 10   |                                |                  | 5                             |      |      | 750                                            | 0.8                               | 17.4 |
| 80                                     | 10   |                                | 5                | 5                             |      |      | 850                                            | 0.8                               | 14.9 |

TABLE 10  
Change rates in the C-value and n-value after test  
(Percent)

| Sample    | 1-watt life test  | 2-watt life test   | Heating cycle test  |
|-----------|-------------------|--------------------|---------------------|
| Example 1 | ΔC: 3%<br>Δn: -5% | ΔC: 5%<br>Δn: -10% | ΔC: 1.5%<br>Δn: -3% |
| Example 2 | ΔC: 1%<br>Δn: -2% | ΔC: 2%<br>Δn: -3%  | ΔC: 1%<br>Δn: -3%   |

TABLE 11

| Fe <sub>2</sub> O <sub>3</sub> | NiO | Ag | Bi <sub>2</sub> O <sub>3</sub> | SiO <sub>2</sub> | B <sub>2</sub> O <sub>3</sub> | CoO | Characteristics of resultant resistors |      |                                      |
|--------------------------------|-----|----|--------------------------------|------------------|-------------------------------|-----|----------------------------------------|------|--------------------------------------|
|                                |     |    |                                |                  |                               |     | C                                      | n    | Changes rates after 2-watt life test |
| 0.1                            | 0.1 | 80 | 14                             | 4                | 1                             | 1   | 4.2                                    | 20.0 | ΔC: 2%, Δn: 4%.                      |
| 0.1                            | 0.1 | 80 | 14                             | 1                | 4                             | 1   | 4.7                                    | 21.4 | ΔC: 3%, Δn: 5%.                      |
| 0.1                            | 0.1 | 80 | 14                             | 1                | 1                             | 4   | 4.9                                    | 23.7 | ΔC: 2%, Δn: 5%.                      |
| 3.0                            | 3.0 | 80 | 14                             | 4                | 1                             | 1   | 5.2                                    | 25.3 | ΔC: 3%, Δn: 3%.                      |
| 3.0                            | 3.0 | 80 | 14                             | 1                | 4                             | 1   | 5.5                                    | 22.4 | ΔC: 3%, Δn: 5%.                      |
| 3.0                            | 3.0 | 80 | 14                             | 1                | 1                             | 4   | 5.4                                    | 23.5 | ΔC: 2%, Δn: 5%.                      |
| 0.1                            | 0.1 | 90 | 7                              | 1                | 1                             | 1   | 4.8                                    | 21.9 | ΔC: 3%, Δn: 5%.                      |
| 0.1                            | 0.1 | 90 | 7                              | 1                | 1                             | 1   | 4.6                                    | 22.6 | ΔC: 3%, Δn: 5%.                      |
| 3.0                            | 0.1 | 90 | 7                              | 1                | 1                             | 1   | 4.4                                    | 23.7 | ΔC: 2%, Δn: 4%.                      |
| 3.0                            | 3.0 | 90 | 7                              | 1                | 1                             | 1   | 4.9                                    | 20.9 | ΔC: 2%, Δn: 3%.                      |
| 1.0                            | 1.0 | 85 | 10                             | 3                | 1                             | 1   | 5.2                                    | 25.3 | ΔC: 2%, Δn: 3%.                      |

What is claimed is:

1. A voltage-nonlinear resistor comprising a sintered wafer consisting essentially of, as a major part, zinc oxide and, as an additive, 0.05 to 10.0 mol. percent of iron oxide and 0.05 to 10.0 mole percent of one member selected from the group consisting of titanium oxide, manganese oxide, barium oxide, strontium oxide, beryllium oxide, and lead fluoride, the opposite surfaces of the wafer both having the same resistance as the material of the wafer, and a silver paint electrode on at least one of the opposite surfaces of said sintered wafer.

2. A voltage-nonlinear resistor as claimed in claim 1, wherein said additive consists essentially of 0.1 to 3.0 mole percent of iron oxide and 0.1 to 3.0 mole percent of one member selected from the group consisting of titanium oxide, manganese oxide, barium oxide, strontium oxide, beryllium oxide, and lead fluoride.

3. A voltage-nonlinear resistor as claimed in claim 1, wherein a silver electrode is on both opposite surfaces of said sintered wafer.

4. A voltage-nonlinear resistor as claimed in claim 1, wherein said silver electrode has a composition of 70.0

wt. percent of silver, 0 to 10 wt. percent of boric oxide, 0 to 10 wt. percent of silicon dioxide, 0 to 60 wt. percent of one oxide selected from the group consisting of cobalt oxide and manganese oxide and 1.0 to 20.0 wt. percent of one oxide selected from the group consisting of bismuth oxide and lead oxide.

5. A voltage-nonlinear resistor as claimed in claim 1, wherein said silver electrode has a composition of 75.0

wt. percent of silver, 0 to 10 wt. percent of boric oxide, 0 to 10 wt. percent of silicon dioxide, 0.05 to 3.0 wt. percent of one oxide selected from the group consisting of cobalt oxide and manganese oxide and 2.95 to 15.0 wt. percent of one oxide selected from the group consisting of bismuth oxide and lead oxide.

## References Cited

## UNITED STATES PATENTS

|           |         |          |         |
|-----------|---------|----------|---------|
| 3,503,029 | 3/1970  | Matsuoka | 252—518 |
| 3,541,029 | 11/1970 | Bowman   | 252—519 |
| 3,515,686 | 6/1970  | Bowman   | 252—518 |

## FOREIGN PATENTS

|    |           |         |               |         |
|----|-----------|---------|---------------|---------|
| 70 | 1,130,108 | 10/1968 | Great Britain | 252—518 |
|----|-----------|---------|---------------|---------|

DOUGLAS J. DRUMMOND, Primary Examiner

U.S. CL. X.R.

75 252—520, 521